# EUROPEAN PATENT APPLICATION

(11) **EP 1 452 242 A2**
(43) Date of publication of application: **01.09.2004**
(21) Application number: 04012916.5
(22) Date of filing: 03.09.1998
(51) Int. Cl.: B05D 3/14, B05D 5/06, B32B 5/14, B32B 15/08, B32B 27/30

(54) **Patterned release finish**

(30) Priority: 08.09.1997 US 58148 P; 01.09.1998 US 144766
(62) Divisional of application: 98948081.9
(71) Applicant: E.I. du Pont de Nemours and Company, Wilmington, DE 19898 (US)
(72) Inventor: Batzar, Kenneth, Cherry Hill New Jersey 08003 (US); Hamilton, Jeffrey Hugh, Greenville Delaware 19807 (US); Rey, Christopher Mark, Hockessin Delaware 19707 (US); Leck, Thomas J, Hockessin Delaware 19707 (US); Herzer, Alan Charles, Turnersville New Jersey 08102 (US)
(74) Representative: Matthews, Derek Peter

(57) **Abstract**

Smooth, patterned substrates useful in producing decorative cookware are formed by coating a base with a mixture of fluoropolymer and magnetic flakes and magnetically inducing an image in the polymer coating composition. The baked fluoropolymer release coating contains magnetizable flakes, a portion of the flakes being oriented in the plane of the substrate and a portions of said flakes being magnetically reoriented to form a pattern in the coating which is observed in reflected light, the flakes having a longest dimension which is greater than the thickness of said coating. The patterned substrate is formed by applying magnetic force through the edges of a magnetizable die positioned under a coated base to induce an imaging effect or pattern. The coating composition in then cured resulting in a smooth surface, patterned nonstick finish on the substrate.

## Description

### REFERENCE TO RELATED APPLICATION

This application claims the benefit of priority of application serial No. 60/058,148, filed September 8, 1997.

### FIELD OF THE INVENTION

This invention relates to non-stick coated article, with a decorative pattern having a three dimensional effect. The instant invention also relates to producing a decorative pattern in coated cookware while maintaining a smooth non-stick surface which allows for easy release of food particles.

### BACKGROUND OF THE INVENTION

It has long been desirable to produce coated cookware which has decorative appeal and maintains good release properties. One attempt to produce patterned cookware which exhibits an illusion of optical depth is described in GB 1,131,038 (Tefal). The specification discloses a process for producing a pattern of flaked magnetic particles in a polytetrafluorethylene (PTFE) matrix as a coating on a substrate. The process is carried out by mixing the flakes with an aqueous dispersion of PTFE and coating the dispersion onto the substrate. After the coating step, a magnet is placed on the underside of the substrate (base), and the magnetic field from the magnet causes the flakes to be attracted toward the magnet. As shown in Figure 3 of the '038 patent, this movement includes the vertical and near vertical orientation of the flakes within the coating thickness and the flakes are entirely contained within the coating, which means that their largest dimension is smaller than the thickness of the coating. This requires either thick coatings or very small flakes (small largest dimension). The problem with small flakes, however, is that they tend not to form a distinguishable pattern in the coating. Consequently, thick PTFE coatings are necessary to produce a visible pattern. Even then, the vertical orientation of the flakes by the magnetic lines of force inevitably causes flakes near the top surface of the coating to protrude from the surface, causing roughness of the baked coating, which is undesirable for a release coating. The '038 patent also discloses that the base has cavities in it, i.e., it has a rough surface, which enables the flakes to be immobilized during the baking of the coating. Among the problems with the magnetic patterning of the release coating by the process of the '038 patent is the need for an excessively thick PTFE coating, which nevertheless fails to completely contain all of the flakes within its thickness and the need for a roughened substrate for adhering the coating to the substrate and immobilizing the flakes during sintering.

Another problem with the pattern formed by the process of the '038 patent is that the pattern is "fuzzy", i.e., lacks clarity. When the coated substrate is placed directly on the magnet of Figure 1 of the '038 patent, the annular pole piece of the magnetic is reproduced in the coating as a toroid ring, deviating from the shape of the circular ring of the pole piece serving as the pattern. When a shaped plate is laid across the top of the magnet, the resultant imprint of the shaped plate is especially fuzzy where the magnetic force is directed through the bulk area of the shaped plate as shown in Figure 2 of the '038 patent. The "fuzzy" image is a manifestation of the of the '038 patent method producing unwanted field lines (magnetic background effects); such method also produces a rough decorative surface. If a stronger magnet is used in the method of the '038 patent, to try to eliminate the fuzziness of the image, i.e. sharpen the image, another unwanted background effect occurs, namely reproduction of the shape of the magnet in the pattern in the coating.

In addition to design, cookware often includes liquid level markings on the inside sidewalls of pots and pans or the like. Traditionally, such markings have been achieved by embossing the metal base prior to overcoating with nonstick finish. However, the depressions protrusions formed by embossing can interfere with the release properties of the surface, causing a buildup of food deposits and becoming a source of corrosion.

### SUMMARY OF THE INVENTION

The present invention in its various embodiments solves the problem of excessive coating thickness while still being able to produce smooth release coatings containing magnetically induced flake patterns within the coating, enables smooth substrates to be used and provides patterns of improved clarity, e.g. line patterns, including novel patterns forming liquid level indicators. In one embodiment, the present invention provides a substrate having a baked release coating thereon which comprises fluoropolymer and magnetizable flakes, a portion of said flakes being oriented in the plane of the substrate and another portion of said flakes having been localized magnetically reoriented from the plane of the substrate, the portion of said flakes which are magnetically reoriented having a different appearance in reflected light than the portion of said flakes oriented in the plane of the substrate, whereby the portion of said flakes which have been magnetically reoriented forms a pattern in said coating, said flakes having their longest dimension being greater than the thickness of said coating.

In the application of the coating composition in liquid form to the substrate, the flakes orient themselves generally parallel to the plane of the surface of the substrate, and the localized magnetic reorientation of the flakes causes the flakes to tilt (reorient) from the original planar orientation. This tilt will vary from perpendicular to the original planar orientation, i.e. perpendicular to the surface of the substrate being coated, to less than perpendicular to the original plane. The planar oriented flakes reflect incident light back to the viewer, while the reoriented flakes do not. Thus, where the magnetic reorientation of the flakes is present in the coating, this gives the appearance of a pattern in the coating. It is important that the flakes be able to reflect light back to the viewer, and this is the reason why large flakes (long dimension greater than the coating thickness) are used. Small flakes are insufficiently reflective to give a distinct difference in appearance between the area of reoriented flakes and planar disposed flakes, or in other words to give a distinct pattern in the coating.

Because of the long dimension of the flakes being greater than the release coating thickness, the reoriented flakes may protrude from the surface of the coating, while the flakes which lie in the plane of the coating, i.e., not tilted, will generally not protrude from the surface of the release coating. Even though some of the reoriented flakes protrude from the surface of the release coating, the protruded portions of such flakes are coated with the composition of the release coating to form "mounds" of release coating encasing the protruding portions of the flakes. The profile of these mounds, tapering into the flat surface of the coating, enable the coating (after baking) to serve as a release coating. By running one's finger over the surface of the baked coating, one can feel that the overall the surface of the patterned release coating is smooth, and that the area of the pattern that appears dark to reflected light, is slightly less smooth than the area that reflects light, but nevertheless serves as a release coating, e.g., releasing food cooked thereon.

In one embodiment of the present invention, the pattern is decorative. When the substrate is cookware or bakeware, the pattern can be present on the cooking (baking) surface and give the appearance of being three dimensional even though the release coating on the substrate is smooth. In a preferred embodiment the release coating is smooth, the smooth surface characterized by a surface roughness of less than 1.5 micrometers. In another embodiment, the pattern is in the form of liquid level indicia in the sidewall of the release-coated vessel. This sidewall marking information is provided by the magnetic reorientation of the flakes without any embossing of the cookware or bakeware sidewall and with the coating containing the magnetically reoriented flakes being sufficiently smooth surfaced to still serve as a release coating.

In another embodiment, the substrate surface is smooth and the coating is adhered to the substrate through a primer layer on the substrate. In a preferred embodiment, the substrate smoothness is characterized by an average surface roughness of less than 1.5 micrometers. In another preferred embodiment, the coating containing the flakes is in two parts. a midcoat layer and a topcoat layer. The flakes are in the midcoat layer and the topcoat can either insure that no flakes protrude from the surface of the overall coating or can smooth out the mounds which encase flakes protruding from the midcoat layer, depending on the thickness of the topcoat. The thickness of the midcoat layer and preferably the combined thickness of the midcoat and topcoat layers is less than the length of the long dimension flakes, in which case while smoothing out the surface of the midcoat, the topcoat will telegraph the tops of the underlying mound through the flat surface of the topcoat. This smoothing out provided by the topcoat further improves the release character of the release coating. If a roughened substrate is used, which does not require a primer layer, the midcoat described above will be the bottom layer or undercoat layer.

The coated substrate of the present invention is preferably made by a process wherein with the application of an aqueous dispersion comprising fluoropolymer and the magnetizable flakes to the substrate, the resultant liquid coating is subjected to localized magnetic force to produce the pattern of reoriented flakes desired. Preferably the aqueous dispersion is applied simultaneously to the substrate with the application of the magnetic force. Another departure from the process of British patent 1,131,038 is how the magnetic force is applied to the flakes, namely from a diffuse magnetic field rather than directly from the magnet itself. The magnet which is the source of the magnetic force is spaced from the substrate being coated. The magnetic force is communicated across the space between the magnet and the flakes in the coating from a diffuse magnetic field intervening between the magnet and the coating through a die of magnetizable material positioned between the diffuse magnetic field and the coating on the substrate. The diffuse magnetic field isolates the coating from direct exposure to the magnetic field of the magnet, eliminating unwanted background effects from the pattern, thereby improving pattern clarity. The magnetizable die has reduced " background effects" on the pattern, i.e., greater clarity, than when the coating is subject to direct exposure of the magnetic field of the magnet. By background effects is meant that the magnetic force operates on flakes lying outside the edges of the desired pattern causing such background flakes to move out of planar configuration. These background effects cause unwanted fuzziness or increased darkness of the pattern edges. Another unwanted background effect is reproduction of the shape of the magnet in the pattern formed in the coating. Thus, in accordance with the present invention, the shape of the pattern can both be sharp and be independent of the shape of the magnet and the pattern can be in the form of lines rather than thick imprints of the source of the magnetic force as in the '038 patent. The magnetizable material can be considered the die for the pattern.

In one embodiment, the die is of sheet metal construction. e.g., forming an annulus, with the "knife" edge of the sheet metal shape (looking like a "cookie cutter") serving as the die. In another embodiment, the die is one or more pins. The edge of the sheet metal die forms a line pattern in the coating corresponding to the shape of the edge (s) of the die. Depending on the spacing of the pins from one another, the ends of the pins form a pattern of disconnected non-reflective or connected non-reflective (lines) regions . Such a configuration of pins is particularly useful for patterning sidewalls which have curved surfaces such as with liquid level markings. In still another embodiment the die can be a plate having a configured edge and/or cut-outs. Instead of the plate being positioned "on-edge" to form the pattern in the coating, a lateral face of the plate is aligned with the bottom of the substrate to be coated, whereby the pattern present in the plate being subjected to the diffuse magnetic field is reproduced in the coating.

### BRIEF DESCRIPTION OF THE DRAWINGS

Figure 1 shows in schematic side elevation an equipment arrangement for forming a magnetically induced pattern in a fluoropolymer release coating on one embodiment of substrate.
Figure 2 is a perspective view of the magnetizable die used to form the pattern in Figure 1.
Figure 3 shows a plan view of the substrate (frying pan) of Figure 1 with the magnetically induced pattern visible in the release coating on the substrate.
Figure 4 shows in side elevation and enlarged cross-section the magnetically reoriented magnetizable flakes deflecting incident light on the release coating to produce the pattern shown in Figure 3.
Figure 5 shows in side elevation and enlarged cross-section a preferred embodiment of the release coating of the present invention.
Figure 6 shows in perspective another embodiment of magnetizable die useful in the present invention
Figure 7 shows in plan view of the substrate the magnetically induced pattern in the release coating obtainable from the die of Figure 6.
Figure 8 shows in plan view another embodiment of magnetizable die for forming a magnetically induced pattern in the form of a liquid level marking in a release coating in accordance with the present invention.
Figure 9 shows in schematic side elevation one use of the die of Figure 8 for forming the liquid level marking in the release coating on the sidewall of the frying pan.
Figure 10 shows in schematic side elevation an equipment arrangement using a configured plate aligned with the underside of a substrate (frying pan) to form a magnetically induced pattern in a fluoropolymer release coating.
Figure 11 shows a plan view of the plate used in the equipment arrangement of Figure 10.
Figure 12 shows a plan view of the substrate of Figure 10 with the magnetically induced pattern visible in the release coating on the release coating.

### DETAILED DESCRIPTION

Reference will now be made in detail to the present invention as illustrated in the accompanying drawings.

In Figure 1 is shown the substrate to be coated and magnetically patterned in accordance with the present invention, the substrate being in the form of a frying pan 2 of non-magnetizable material such as aluminum, copper, stainless steel, glass or ceramic. The frying pan 2 is shown to have a handle 4. A liquid dispersion of a mixture of fluoropolymer resin and magnetizable flakes is applied as a spray 6 onto the interior surface of the frying pan 2 to form a release coating 8 thereon as best shown in Figure 4. The flakes 10 in the sprayed composition tend to orient themselves generally parallel to the surface of the substrate as shown in Figure 4, except in the region of magnetic force applied by magnetic die 12, which causes the flakes 10' in such region to reorient out of the plane of the substrate, i.e., such flakes form an angle with the plane of the substrate, whereby incident light on the release coating either is reflected at an angle away from the perpendicular path of the incident light as shown in Figure 4 or is not reflected at all when the reoriented flakes are parallel to the incident light. The flakes 10' which are tilted to the perpendicular or near perpendicular protrude from the surface of layer 8, but the protruding portions of the flakes are encased in release composition of which layer 8 is composed to formed small mounds 11 of release coating protruding from the otherwise flat surface of the coating 8. Where the flakes 10 are parallel to the surface of the substrate, the incident light is reflected directly back to the viewer. The difference in reflection of the incident light gives the release coating a magnetically induced pattern in the shape of the magnetizable die.

The magnetic force is applied to form the pattern as further shown in Figure 1. The magnetizable die 12 is made of sheet metal, e.g., 0.1 mm to 4 mm thick, and is in the form of a morningstar pattern as best shown in Figure 2. The sheet metal forming the die 12 is at an angle with respect to the plane of the underside of the fry pan 2. so that the upper edge and not the face (side) of the sheet metal forms the pattern of localized magnetic force in the coating 8. The upper edge of the sheet metal can be as thin as a knife edge as well as thicker, e.g., up to the 4 mm thickness mentioned above. The die 12 in essence looks like a cookie cutter, with its size depending on the size of the pattern to be formed in the release coating. In order to stabilize the sheet metal walls forming the die, the interior space 14 of the die can be filled in by nonmagnetizable solid material such as wood (not shown).

The magnetizable die is not the source of the magnetic force. Instead, the source of the magnetic force is magnet 16 which can be a permanent magnet or as shown in Figure 1 can be an electromagnet having a central pole 18 surrounded by electrical coil 20 and in turn by an annular pole 21. The magnet 16 generates the magnetic force necessary for the invention. The magnet 16 is spaced from the frying pan 2, and the magnetic force from the magnet is communicated to the release coating through the die 12. The spacing of the magnet from the underside of the substrate can be great enough that the coating on the substrate is not directly exposed to the magnetic force of the magnet or the magnetic force of the magnet 16 is diffused into a magnetizable metal plate 22 interposed between the magnet 16 and die 12. In either case, the die communicates the magnetic force from a diffuse magnetic field rather than the coating 8 being exposed directly to the magnetic field of the magnet. This enables the magnetically induced pattern in the release coating to be precisely controlled by the configuration of the magnetizable die 12, wherein the pattern closely conforms to the shape of the die facing the underside of the substrate. The momingstar pattern 24 as a hollow line pattern in the release coating resulting from the use of die 12 is shown in the base of the frying pan 2 in Figure 3. This pattern is visible to the naked eye by virtue of light being reflected from the surface of the release coating, i.e. from the surface inside and outside the pattern.

Application of the magnetic force to the flakes in the release coating through the magnetizable die such as die 12 is effective to localize the reorientation effect on the flakes in the coating composition to provide the faithful reproduction of the die. The flakes are assumed to be reoriented, because in the absence of magnetic force, the flakes will be oriented substantially in the plane of the coating, so as to be light reflective. The magnetic force is not so strong that the die itself creates unwanted background fuzziness in the pattern, but is strong enough to produce the pattern in the coating. The diffuser plate 22 also enables the magnet to be any size, i.e. independent of the size of the pattern to be magnetically induced in the release coating, except that the area of the face of the magnet should be smaller, and totally contained within, the area of the diffuser plate, so that lines of force of the magnet cannot pass directly to the substrate being coated. Thus, one size magnet can be used to create a wide variety of pattern sizes and shapes, depending on the magnetizable die used.

A key to producing cookware which is both decorative and still retains its release properties is proper modulation of the magnetic force applied to the release coating by the die. Such modulation can be achieved by the height of the magnetic die and/or by use of the diffuser plate and can be facilitated by including additional spatial gaps of non-magnetizable material as needed to produce the pattern effects desired. Such a gap can be achieved by using nonmagnetizable spacing sheets (not shown) between the diffuser plate and the die or the magnetic die can be spaced from the underside of the frying pan instead of being in contact therewith as shown in Figure 1. Another spatial gap can be achieved by the thickness of the cookware substrate thereby instituting a gap between the tips of the magnetizable die and the magnetizable flakes in the release coating. Any gap in addition to the thickness of the substrate (uncoated frying pan), spacing of the die from the substrate and/or the diffuser plate is selected to eliminate background effects of the magnetic field of the magnet, while allowing the magnetic force to penetrate the gap and via the magnetic die, to act on the release coating.

In the case of point and edge effects, field strength has been determined to drop by a factor of 1/d⁷ where d is the distance of the spatial gap between the tips of the magnetizable die and the magnetizable flakes. So even a small spatial gap will greatly affect the magnetic strength By reducing the strength of the magnetic field and eliminating or decreasing certain lines of force, magnetic background effects are reduced. This results in a smooth decorative surface on the substrate.

While the magnetizable flakes still in the liquid state of the coating are mobile, it has been found that clarity of the pattern is improved when the coating is exposed to the magnetic force from the magnetizable die simultaneously with the step of applying the liquid coating composition to the substrate. To facilitate these steps being carried out simultaneously, the magnetic die is preferably positioned on the underside side of the substrate to be coated with the release coating instead of on the coating side thereof.

The resultant liquid coating, containing the magnetically-induced pattern, is then dried and baked to sinter or otherwise fuse the fluoropolymer to form the release coating, by heating the coating typically to temperatures of 350°C to 420°C, depending on the fluoropolymer resin used. The flakes in the release coating should be made of material that while magnetizable, are unaffected by such heating. Examples of material from which the flakes can be made include such metals as iron and nickel and alloys containing these metals, with stainless steel being the preferred material. For simplicity, the fluoropolymer resin/flake coating is referred to as a release coating both before and after the baking step. when in,fact the baking step is necessary before the release (non-stick) characteristic is realized.

The baking stabilizes (affixes) the magnetically induced pattern of reoriented flakes within the release coating on the substrate. The substrate can be roughened such as by grit blasting or chemical etching to create cavities to which the release coating can anchor. Preferably, however, the substrate as shown for the frying pan 2 surface in Figure 4 is smooth. Even when smooth, the magnetically induced pattern of reoriented flakes obtained in accordance with the present invention remains in place during the baking process, whereupon the pattern becomes permanent within the coating. In accordance with the preference for a smooth surfaced substrate, the release coating is preferably adhered to the substrate via an intervening primer layer 30 such as shown in Figure 5. In another preferred form of the present invention, the release layer or coating is in two parts (layers), the layer 8 which contains the flakes 10, and a topcoat 32 which is free of such flakes. The layer 8 is thereby present as a midcoat. The topcoat 32 contains minute mounds 33 extending from its surface, telegraphing the presence of the mounds 11 from layer 8, but smoothing them out. The presence of the topcoat 32 thus provides a smoother exposed surface for the release coating, and if thick enough can mask the mounds 11 in the underlying layer altogether. The topcoat adds to the aesthetics of the decorative surface by improving the gloss.

Figure 6 shows another embodiment of magnetizable die 40 comprising a wooden plate 42 having holes drilled therein to accommodate magnetizable metal pins 44 which are preferably tightly engaged in their respective holes. This die can be used in place of die 12, with the bottom ends of the pins in contact with the diffuser plate 22 and the top ends in contact with (or adjacent to) the underside of the frying pan 38 which is similar to frying pan 2. Each pin, being at an angle to the plane of the underside of the frying pan 38, communicates the magnetic force from the diffuse magnetic field of the plate 22 to the coating to form a pattern visible in reflected light as a plurality of dark points (dots) 45 within the a light-appearing coating, with the diameter of the dots in the pattern being slightly larger than the diameter of the rods pins as shown in Figure 7. The pattern (placement and frequency) of pins can be varied as desired and can be combined with an annular pattern such as that momingstar pattern shown in Figure 3. The dots formed within the coating can have the optical appearance of depressions lending an impression of optical depth and therefore thickness to the cookware article, while yet retaining a smooth, nonstick surface. For convenience, the structure forming the magnetic die, e.g. the sheet metal forming the die in Figure 2 or the pins 44, will be positioned perpendicular, i.e. the die itself can be considered as being perpendicular, to this plane of the underside of the substrate bearing the liquid coating composition.

Figure 8 shows in enlarged plan view another embodiment of a magnetizable die 46 based on pins 48. In this embodiment, the pins are of smaller diameter, e.g. 1 mm in diameter as compared to 3 mm in diameter for the pins 44 of Figure 6. The pins 48 are spaced closely together, e.g. pin heads are in close proximity or touching contact with each other but can be held in place the same way, namely by a wooden plate or foam block, 50, having holes which tightly accommodate the pins 48. As shown in Figure 8, the pins 48 form information instead of decoration, namely to show a liquid level and label of "1 CUP" for the liquid level. This die can be used to apply this information to the sidewall of the frying pan 38, or other release coated vessel, such as shown in Fig 9, wherein the die is shown positioning its pins against the sidewall of the frying pan and against diffuser plate 52, beneath which is the magnet 54 which is the source of the magnet force reaching the flakes in the coating composition. The close spacing of the pins 48 creates a pattern of continuous lines in the coating, providing volume information appearing on the frying pan without any indentation being present in the substrate forming the frying pan or without any change in smoothness of the release coating which contains this liquid level indicia. In this embodiment, the pins 48 can be made in different lengths to account for the curvature of the sidewall of the frying pan. This embodiment of die can also be made of sheet metal formed in the pattern of information desired and held in place by a wooden base or foam block. The use of pins, however, as in Figures 8 and 9 facilitates the forming of a wide variety of patterns of indicia, such as additional liquid level markings, including letter description thereof, e.g. oz. or ml. The pins used as the magnetic die in the present invention can have any diameter desired depending on the pattern desired, but typically, they will have a diameter of 0.5 mm to 5mm.

Figures 10-12 show a different embodiment, wherein the magnetically indiced pattern in the release coating is formed using a configured plate. the face of which is oriented in the same direction as the bottom of the substrate to be coated. In Figure 10, the configured plate 60 of magnetizable material is positioned in contact with the bottom surface of frying pan 62 which is similar to frying pan 2. Instead of diffuser plate 22 used in Figure 1, a diffuser block 64 of magnetizable material is used, and a magnet 66 is positioned beneath block 64. The height of block 64 is such that for the strength of the magnet 66 used, sufficient magnetic force reaches the magnetizable flakes in the release coating (while still flowable) to cause the flakes to orient away from the plane of the substrate so as to reproduce the pattern of plate 60. While Figure 10 shows the under-surface of the frying pan, the plate 60, block 64, and magnet 66 all being in sequential contact with one another. an air gap or non-magnetizable spacer can be introduced between any on the elements forming this equipment arrangement, so as to modulate the magnetic force emanating from the magnet. Such modulation can be used for example if it is desired for space reasons to use a diffuser plate like that of Figure 1 instead of block 64. The area of the face of magnet 66 is smaller than the bottom area of the diffuser block 64, and the magnet is positioned within the bottom area of the diffuser block, so that all of the magnetic force reaching the plate 60 does so by passage through the block 64. Figure 11 shows the configuration of the edge of plate 60, consisting of a solid center region 68 having tapering arms 70 radially extending therefrom. Preferably the diffuser block which is in this embodiment an upstanding cylinder, because the plate is derived from a circular plate, has an outer diameter which is about the same as the diameter of the region constituting the solid center 68 of the plate 62. The pattern 72 of configured plate 60 is reproduced magnetically in the release coating on the cooking surface of frying pan 62 as shown in Figure 12 as a dark region corresponding to the pattern of plate 60 surrounded by a light region, with the dark region appearing to be recessed below the light region, giving the cooking surface of the frying pan a three dimensional appearance. Other configurations which depart from a circular pattern from which the plate 60 is derived can be used

Heat resistant materials especially useful in forming the primer layer and the release coating in clude fluoropolymer resin components. Such resin contains at least 35 wt% fluorine. One particularly useful fluoropolymer is polytetrafluoroethylene (PTFE) which provides the highest heat stability among the fluoropolymers. Optionally, the PTFE contains a small amount of comonomer modifier which improves film-forming capability during baking, such as perfluoroolefin, notably hexafluoropropylene (HFP) or perfluoro(alkyl vinyl) ether (PAVE), notably wherein the alkyl group contains 1-5 carbon atoms, with perfluoro(ethyl or propyl vinyl ether) (PEVE and PPVE, respectively) being preferred. The amount of modifier may be insufficient to confer melt-fabricability to the PTFE, generally no more than about 0.5 mole%. The PTFE, can have a single melt viscosity, usually about 1 x 10⁹ Pa.s, but, if desired, a mixture comprising PTFE's having different melt viscosities can be used to form the fluoropolymer component.

In one aspect of this invention, the fluoropolymer component, is melt fabricable fluoropolymer, either blended with the PTFE, or in place thereof. Examples of such melt- fabricable fluoropolymers include tetrafluoroethylene (TFE) copolymers with one or more of the comonomers as described above for the modified PTFE but having sufficient comonomer content to reduce the melting point significantly below that of PTFE. Commonly available melt-fabricable TFE copolymers include FEP (TFE/HFP copolymer) and PFA (TFE/PAVE copolymer), notably TFE/PPVE copolymer. The molecular weight of the melt-fabricable tetrafluoroethylene copolymers is sufficient to be film-forming and be able to sustain a molded shape so as to have integrity in the primer application. Typically, the melt viscosity of FEP and PFA will be at least about I x 10² Pa.s and may range to about 10 - 400 x 10³ Pa.s as determined at 372°C according to ASTM D-1238.

The fluoropolymer component is generally commercially available as a dispersion of the polymer in water, which is the preferred form of the composition for this invention for ease of application and environmental acceptability. By "dispersion" it is meant that the fluoropolymer particles are stably dispersed in an aqueous medium, so that settling of the particles does not occur within the time when the dispersion will be used. The stability of the dispersion can be achieved as the result of the relatively small size of the fluoropolymer particles, typically on the order of 0.2 micrometers, and the use of one or more surfactants in the aqueous dispersion. Such dispersions can be obtained directly by the process known as dispersion polymerization, optionally followed by concentration and/or further addition of surfactant. Examples of suitable surfactants include at least one of octylphenoxytriethoxyethanol, triethanolamine oleate, among others.

The release coating, which in one embodiment may be a midcoat and a topcoat, used in this invention is generally derived from a dispersion of one or more fluoropolymers to which has optionally been added a dispersion of an acrylic polymer. Suitable midcoat and topcoat are described by U.S. Patent Nos. 4,180,609 (Vassiliou); 4,118,537 (Vary & Vassiliou); 4,123,401 (Berghmans & Vary); 4,351,882 (Concannon) hereby incorporated by reference.

The composition forming the midcoat and topcoat used in the present invention can contain in addition to the fluoropolymer component, a dispersion of a polymer of monoethylenically unsaturated monomers, such as the acrylic polymer dispersions described in U.S. Patent Nos. 4,123,401 (Berghmans and Vary) and 4,118,537 (Vary and Vasilliou); hereby incorporated by reference. The coating composition typically shows improved coalescence on curing if a polymer of monoethylenically unsaturated monomers have been added to the fluoropolymer component. The polymer of monoethylenically unsaturated monomers can be any suitable polymer or copolymer (in the sense of being composed of two or more types of monomers) of ethylenically unsaturated monomers which depolymerize. and whose depolymerization products vaporize, in the temperature range of about 150°C below the fusion temperature of the fluoropolymer used to about the fluoropolymer's decomposition temperature and thus vaporizes during the baking step. It may be desirable that the polymer of monoethylenically unsaturated monomers be in solution in a solvent compatible with the rest of the system or be present as a stable dispersion of small particles. For desired results, the average particle size is generally below 1 micrometer.

Illustrative of acrylic polymers which can be used as an additive are polymers of one or more monoethylenically unsaturated monomers which also contain one or more monoethylenically unsaturated acid units. Representative of the monomers are alkyl acrylates and methacrylates having 1-8 carbon atoms in the alkyl group, styrene, alpha-methyl styrene and vinyl toluene. Representative of the acid units are acrylic acid, methacrylic acid, fumaric acid, itaconic acid and maleic acid (or anhydride). Mixtures of these polymers can also be used. The acid units of these polymers can optionally be esterified with glycidal esters of 4-14 carbon atoms. Such a polymer is ordinarily present at a concentration of about 2-300% by weight of the fluoropolymer, and preferably about 5-20%. The preferred polymer additive is an acrylic latex of a methylmethacrylate/ethylacrylate/methacrylic acid 39/57/4 terpolymer.

The release coat, in particular the midcoat used in the present invention, contains an effective amount of light reflecting magnetizable flakes to produce a pattern in the coating upon localized reorientation of the flakes. The release coating generally contains from 2 - 6 wt. % of magnetizable flakes, based on the dry weight of the coating composition. Some of these flakes may have a longest dimension which is less than the thickness of the coating, e.g., less than 50 wt. % of the flakes, but this condition may exist because of the flake size distribution in the flakes that are commercially available. The "short" flakes make little contribution to the visibility of the pattern. Particularly useful are 316L stainless steel flakes having an average longest dimension of from 20 to 60 micrometers, and normally, the flakes will be a mixture of sizes in which a substantial proportion, preferably at least 40 wt%, has a longest dimension of at least 44 micrometers.

The compositions forming the primer, intermediate and top coatings used in the present invention often contain one or more pigments, normally in a mill base medium that is either soluble in or miscible with the water of the fluoropolymer aqueous dispersion. However, judicious care is needed in selecting the pigment and quantities of pigment for use in the midcoat and topcoat used in this invention in order not to mask the pattern created by magnetic induction. The pigment mill base is normally produced by milling (grinding) pigment in its liquid medium, which deagglomerates the pigment and produces dispersion uniformity. The preferred medium is water which contains an amount of a surfactant sufficient for the mill base to become an aqueous dispersion of the pigment by the milling process. Pigments for use in cookware applications have limitations imposed on their use by the U.S. Food and Drug Administration (FDA) because of food contact. Pigments to be used in this invention must be heat stable and nontoxic. Suitable pigments include at least one member from the group of carbon black, titanium dioxide, iron oxide, and zeolites such as ultramarine blue, cobalt blue, among others.

The compositions forming the topcoat when used in this invention often contain mica particles, and mica particles coated with pigment. Such particles impart scratch resistance to the articles on which they are coated. These particles have an average longest dimension of about 10 to 200 micrometers, preferably 15-50 micrometers , with no more than 50% of the particles of flake having longest dimensions of more than about 500 micrometers. For use in this invention, mica particles coated with pigment having a longest dimension of 1-15 micrometers are preferred. Small particle size mica flakes, whether present in the coating which contains the flakes and/or in the topcoat when used, allow the magnetically induced pattern to be seen without scattering light or showing metallic luster, yet provide reinforcement for the topcoat. The mica particles coated with pigment preferred for this invention are those described in U. S. Patent Nos. 3,087,827 (Klenke and Stratton); 3,087,828 (Linton); and 3,087,829 (Linton); hereby incorporated by reference. The micas described in these patents are coated with oxides or hydrous oxides of titanium, zirconium, aluminum, zinc, antimony, tin, iron, copper, nickel, cobalt, chromium, or vanadium. Titanium dioxide coated mica is preferred because of its availability. Mixtures of coated micas can also be used. The mica or coated mica is ordinarily present in the topcoat at a concentration of about 0.2-20% by dry weight of the composition.

The primer coating when used in this invention is generally derived from an aqueous dispersion of at least one fluoropolymer and a water soluble or water dispersible film-forming binder material. A suitable primer is described by the ,US Patent Nos. 4,087,394 (Concannon); 5,240,775 (Tannenbaum) and 5,562,991 (Tannenbaum); hereby incorporated by reference.

The film-forming binder component that can be used in forming the primer coating is composed of polymer which is thermally stable. This component is well known in primer applications for non-stick finishes. for adhering the fluoropolymer-containing primer layer to substrates and for film-forming within and as part of the primer layer. The binder is generally non-fluorine containing and yet adheres to the fluoropolymer. Preferred binders are those that are soluble or solubilized in water or a mixture of water and organic solvent for the binder. which solvent is miscible with water. This solubility aids in the blending of the binder with the fluorocarbon component in the aqueous dispersion form. An example of the binder component is polyamic acid salt which converts to polayamideimide upon baking of the composition to form the primer layer. This binder is preferred because in the fully imidized form obtained by baking the polyamic acid salt, this binder has a continuous service temperature in excess of about 250°C. The polyamic acid salt is generally available as polyamic acid having an inherent viscosity of at about 0.1 as measured as a 0.5 wt % solution in N,N-dimethylacetamide at about 30°C. It is dissolved in a coalescing agent, such as N-methylpyrrolidone, and a viscosity-reducing agent, such as furfuryl alcohol and reacted with tertiary amine, preferably triethylamine, to form the salt, which is soluble in water, as described in greater detail in U.S. Patent Nos. 4,014,834 (Concannon) and 4,087,394 (Concannon); the disclosure of both is hereby incorporated by reference. The resultant reaction medium containing the polyamic acid salt can then be blended with the fluoropolymer aqueous dispersion, and because the coalescing agent and viscosity-reducing agent are miscible in water, the blending produces a substantially uniform coating composition. The blending can be achieved by simple mixing of the liquids together without using excess agitation so as to avoid coagulation of the fluoropolymer aqueous dispersion. The proportion of fluoropolymer and binder in compositions of the present invention can be in the weight ratios of about 0.5 to 2.5:1. The weight ratios of fluoropolymer to binder disclosed herein are based on the dry weight of these components in the primer layer, which in essence is the same as the relative weight in the primer layer after baking the composition after application as a coating to a substrate. When the composition of the invention is in the preferred aqueous form, these components will constitute about 5 to 50 wt. % of the total dispersion.

An inorganic filler film hardener component may be present in the primer composition. The film hardener is one or more filler type materials which are inert with respect to the other components of the composition and thermally stable at baking temperatures which fuse the fluoropolymer and binder. Preferably the film hardener is water insoluble so that it is uniformly dispersible but not dissolved in an aqueous dispersion. By filler-type material is meant that the filler is finely divided, generally having a particle size of about 1 to 200 micrometers. usually 2 to 20 micrometers, which is usually obtained by the film hardener component and which imparts durability to the primer layer by resisting penetration of sharp objects that may penetrate the fluoropolymer overcoat.

Examples of the film hardener include one or more metal silicate compounds such as aluminum silicate and metal oxides, such as, titanium dioxide and aluminum oxide. Examples of such film hardeners are described in U.S. Patent 5,562,991 (Tannenbaum) and U.S. Patent No. 5,250,356 (Batzar); the disclosure of which is hereby incorporated by reference.

The primer composition used in the present invention in aqueous dispersion form may also contain such other additives as adhesion promoters, such as colloidal silica or a phosphate compound, such as a metal phosphate, e.g., Zn, Mn, or Fe phosphate.

The coatings used in the present invention, whether single coating containing the magnetizable flakes, or multiple coatings, such as primer, midcoat (containing the flakes) and topcoat, can be applied to substrates by a variety of techniques and to a variety of substrates. Roller, dip, and spray coating can be utilized. It is only necessary that the coating composition which contains the magnetizable flakes be applied as a liquid composition so that the flakes can be localized magnetically reoriented to form the pattern. The layer containing the magnetizable flakes will be thinner than the longest dimension of the flakes and will generally be 5-40 micrometers thick, preferably 5-30 micrometers thick, more preferably 5-25 micrometers thick (0.2-1 mil). When the release coating is a combination of midcoat (containing the flakes) or undercoat and topcoat, the combined thickness will generally be 5-50 micrometers thick, preferably 5-40 micrometers thick. Preferably, the flake-containing layer will be the thicker layer, constituting 60 to 90% of the total thickness of the to layers, and more preferably 70 to 85%. The magnetizable flakes are chosen to have a longest dimension which is greater than the thickness of the flake-containing layer, and more often, thicker than the total thickness of the flake-containing layer and the topcoat, if present. The primer layer, if used will generally have a thickness of 0.5 to 10 micrometers, more often 5 to 10 micrometers (0.2-0.4 mils). The layer thicknesses disclosed herein refer to the dry film thickness (DFT).

The substrates can be any non-magnetizable material which can withstand the relatively high bake temperatures used to fuse the coatings. Such substrate materials include metals and ceramics, such as aluminum, anodized aluminum, stainless steel, enamel, glass, pyroceram, among others. The substrate can be gritblasted (roughened) or smooth, and cleaned prior to coating. For pyroceram and some glass, improved results are obtained by activation of the substrate surface such as by slight, chemical etch, which is not visible to the naked eye. The substrate can also be chemically treated with an adhesion agent such as the mist coat of polyamic acid salt disclosed in U.S. Patent No. 5,079,073 (Tannenbaum); hereby incorporated by reference.

The compositions described above are particularly used to provide an article of cookware, having a cooking surface which comprises a multi-layer, non-stick coating on a substrate which coating minimizes sticking by food residues and which is heat resisting by being stable above about 300°C. The present invention provides for a coated substrate having a magnetically induced image pattern and preferably having an average surface roughness,(abbreviated Ra), less than 1.5 micrometers. as determined using a Hommel Profilometer, model T-500. Typically, the surface roughness will be at least 0.5 micrometers. The substrate itself preferably has the same smoothness, preferably less than 1.5 micrometers and more preferably less than 1.25 micrometers.The coated substrate of the present invention may be in the form of numerous articles of decorative cookware such as frypans, pots, bakeware, casseroles and the like. Although items of cookware are herein illustrated, numerous other household or industrial applications of this technology are contemplated. By example, the sole plate of an iron may be provided with a magnetically induced pattern. Processing tanks or vats having a release finish may benefit from liquid level marking or the like. Further, industrial coaters may choose to apply identification markings or a logo to release coated surfaces by the disclosed magnetic inducing techniques.

### EXAMPLE 1

A pattern is magnetically induced in a release coating on an aluminum substrate which has the form of a frying pan. The setup for applying the coating is similar to that illustrated in Figure 1

Aluminum frying pan 2 has a diameter of 25.4 cm and is typically 1.5 -3.2 mm thick. The frying pan is positioned over a magnetizable die 12 which is akin to a mold or "cookie cutter" being formed from magnetizable sheet metal into a morning star pattern as shown in Figure 2. The die is formed from 1010 steel alloy sheet of 1.6 mm thickness. The die has a pattern of an 8 pointed star having an apparent diameter of 22.9 cm inches with edges that are 10 cm high.

The magnetizable die 12 is positioned over a diffuser plate 22 which rests on a platform 9 (not shown). The plate is a carbon steel plate having the dimensions of 30.5 x 30.5 x 0.65 cm. Positioned between the diffuser plate 22 and the magnetizable die 22 are two nonmagnetizable spacer sheets (not shown) of aluminum having the dimensions 30.5 x 30.5 x 1.3 cm. The platform is positioned over magnet 16 and provides a shield between diffuser plate 22 and magnet 16 and prevents plate 22 from adhering to the magnet. Magnet 16 is a permanent magnet of Neodimium-Iron- Boron Alloy of 10 cm diameter with a capability of generating 2 tesla (20,000 gauss) manufactured by Dexter Magnetics of Sunnyvale, CA 94086. Diffuser plate 22 absorbs upwardly emanating magnetic fields and drives the fields horizontally creating a larger workable magnetic area equal to the breadth of the diffuser plate, but of weakened magnetic force.

The additional nonmagnetizable aluminum spacer sheets further dampen the strength of the magnetic field acting on magnetizable flakes 10' in release coating 8 as the coating is applied to frypan 2. The distance between magnet 16 and magnetizable die 12 as illustrated in Figure 1 may be adjusted to deliver the magnetic force of desired strength through the edges of die 12. The magnetic force as measured at the tip of the magnetic die in contact with the frypan is 128 gauss. It has been found that by reducing the strength of the magnetic field and eliminating or decreasing certain lines of force, that magnetic background effects are reduced. This results in a decorative surface on the substrate that is smooth.

A primer having the composition of Table 1 is sprayed on a clean, lightly etched aluminum frying pan having a surface smoothness of 1.25 micrometers to dry film thickness (DFT) of 15 micrometers. The primer was dried at 66°C for 5 minutes. A midcoat with magnetizable flakes having the composition of Table 2 is sprayed onto the frying pan to a DFT (dry film thickness) of 13 micrometers as magnetic force was applied through the magnetizable die in accordance with the present invention, causing a portion of the flakes to magnetically reorient into the pattern of the edges of the die. A topcoat having the composition of Table 3 is sprayed over the midcoat to a DFT of 13 micrometers while the midcoat is still wet also in the presence of magnetic force. The entire system is baked at 427°C to 435°C for 5 minutes. The frying pan has a decorative surface with a magnetically induced pattern and an average surface roughness, (Ra) less than 1.5 micrometers , as determined using a Hommel Profilometer, model T-500.

In all of the following Tables: "solvent-surfactant blend" corresponded to approximately 19.5% butyl carbitol, 23.9% mixed aromatic hydrocarbons, 4.7% cerium octoate, 37% triethanolamine, 8% lauryl sulfate, and the balance was water; and "acrylic dispersion" corresponded to approximately 39/57/4 methyl methacrylate/ethyl acrylate/methacrylic acid. The polymer comprised about 40% of the dispersion, 9% triethanolamine, 8% sodium lauryl sulfate, and the balance was water.

**TABLE 1**

| **Primer** | **Coating Composition (Wt. %)** | **Solids Content in Finished Article (Wt. %)** |
|---|---|---|
| Furfuryl Alcohol | 1.85 | - |
| Polyamic acid salt in N-Methyl Pyrrolidone | 18.3 | 30.39 |
| Deionized Water | 48.8 | - |
| Mica | 0.050 | 0.03 |
| PTFE Dispersion | 8.04 | 27.38 |
| FEP Dispersion | 5.95 | 18.10 |
| Colloidal Silica Dispersion | 3.64 | 6.01 |
| Carbon black dispersion | 8.09 | 13.43 |
| Aluminum silicate dispersion | 5.25 | 4.64 |

**TABLE 2**

| **Intermediate** | **Coating Composition (Wt. %)** | **Solids Content in Finished Article (Wt. %)** |
|---|---|---|
| PTFE Dispersion | 58.5 | 81.0 |
| PFA Dispersion | 10.6 | 14.7 |
| Deionized Water | 3.2 | - |
| 316L SS Flake* | 1.9 | 4.3 |
| Solvent-Surfactant blend | 13.1 | - |
| Acrylic polymer dispersion | 12.7 | - |

| | | |
|---|---|---|
| *SS Fine water grade, -325 mesh with a D-50 = 25 microns (more than 50% of the particles have a longest dimension of at least 25 microns) produced by Novamet Specialty Products of Wyckoff, N.J. | | |

**TABLE 3**

| **Topcoat** | **Coating Composition (Wt. %)** | **Solids Content in Finished Article (Wt. %)** |
|---|---|---|
| PTFE Dispersion | 66.95 | 94.55 |
| PFA Dispersion | 3.51 | 4.96 |
| Deionized Water | 3.77 | - |
| Mica (1-15 microns) | 0.21 | 0.49 |
| Solvent-Surfactant Blend | 12.51 | - |
| Acrylic polymer dispersion | 13.04 | - |

### EXAMPLE 2

A pattern is magnetically induced in a release coating on an aluminum substrate which has the form of the sidewall of a frying pan. The setup for applying the coating is similar to that illustrated in Figure 9.

Aluminum fry pan 38 has a diameter of 25.4 cm and is typically 1.5 -3.2 mm thick. The fry pan is positioned over a magnetizable die 46 based on pins 48 wherein the die is positioned against the sidewall of the frypan and against diffuser plate 52 beneath which is placed magnet 54. as shown in Figure 8. The die is formed from a plurality of straight pins of steel alloy having a 1 mm diameter head and a length of 3 cm. The pins are spaced closely together, e.g. pin heads are in touching contact with each other and are held in place by a foam block 50 of polystyrene of 1.95 cm thickness which tightly accommodates the pins . The pin heads are positioned flush to one surface of the foam block and in contact with the frypan. The pin ends protrude through the opposite surface of the foam block and are in contact with the diffuser plate. The die is a pattern of liquid level marking "1 CUP".

The platform, diffuser plate and magnet are the same as those specified in Example 1. No spacer plates are present. Preparation of the frying pan, compositions of primer, midcoat, and topcoat. and method of application are the same as those specified for Example 1.

The close spacing of the pins 48 creates a pattern of continuous lines in the coating, providing liquid level markings appearing on the frying pan without any indentation being present in the substrate forming the frying pan or without any change in smoothness of the release coating which contains this liquid level indicia.

### EXAMPLE 3

Similar to example 1, two aluminum frying pans, but of differing thicknesses, are coated with a magnetically induced pattern. One frying pan is 8 gauge, e.g., 3.2 mm, the other pan is 6 gauge, e.g., 4.1 mm. Using fry pans of different thicknesses illustrates the differences of varying the spatial gap between the tip of die and the magnetizable flake in the release coating. The die for this Example 3 is formed by positioning sheets from 1010 steel alloy of 1.6 mm thickness x 10 cm x 6.9 cm in alternating arrangement with sheets of 1.6 mm x 10cm x 5.7 cm inches in tightly fitting slots of a foam block to form 12 radiating edges that form a pattern of radiating lines (similar to the line representation of a sun) with an apparent diameter of 17.8 cm . The edges of one side of the die are positioned against the frying pan bottom with opposite edges of the die positioned against the diffuser plate. The spatial gap between the tips of the die and the magnetizable flakes differ by the thickness of the two frying pans.

The platform, diffuser plate and magnet are the same as those specified in Example 1. No aluminum spacer plates are present. Preparation of the frying pan, compositions of primer, midcoat, and topcoat, and method of application are the same as those specified for Example 1. The magnetic force as measured at the tip of the magnetic die in contact with the frying pan is 300 gauss.

Radiating line patterns are visible in both frying pans. However, the pattern as determined by visual inspection, in the thicker (6 gauge) pan is somewhat weak, yet has lines of greater clarity (less fuzzy) due to the increased spatial gap. The pattern created in the thinner (8 gauge) pan is strong but the lines are fuzzy. To correct the pattern in the thicker pan, a larger (stronger) magnet which can produce a stronger magnetic force communicated to the coating by the magnetic die is used. To correct the pattern in the thinner pan, spacer plates are used to modulate the magnetic force delivered to the die.

### EXAMPLE 4 (Comparative)

Similar to Example 1, an aluminum frying pan, is coated with a magnetically induced pattern but instead of the set up as described in Fig 1 herein, a pole piece in the form a of a shaped plate of magnetizable steel (8mm thick) having the same morning star pattern is placed directly on (laid across) the magnet. The shaped plate is in contact with the underside of the frying pan. The pole piece is a flat plate with no hollow interior, and serves as a template akin to a "dress pattern" used for sewing. The magnetic force is directed through the bulk area of magnetic template acting on the magnetizable flakes of the release coating. The magnetic force is sufficient to cause orientation of the flakes but not excessive to obliterate the resultant pattern. Nevertheless, directing magnetic force the bulk area produces unwanted field lines which result in a fuzzy outline to the solid magnetic imprint and a roughened decorative surface on nonmagnetic base 1. The roughened surface is unsuitable in that food particles tend to stick. Further the surface is more susceptible to gouging because of flake has oriented on an angle and is more likely to respond to be pulled from the coating.

The magnet used is 0.6 tesla (600 gauss), permanent magnet. No platform, diffuser plate or spacer plate is present. Preparation of the frying pan, compositions of primer, midcoat, and topcoat, method of application and thickness of coatings are the same as those specified for Example 1. The magnetic force of the die in contact with the frying pan measured as follows: at the point of the star, 300 gauss; at the edge of the star, 180 gauss; at the interior of the pattern. 120 gauss.

The frying pan has a decorative surface with a magnetically induced pattern and an average surface roughness, (Ra), of between 1.5 - 3.0 micrometers.

### EXAMPLE 5

In this Example, the equipment arrangement shown in Figs, 10-12 is used. using a frying pan similar to that used in Example 1 having a smooth interior surface. The magnetizable die is the configured plate of Figure 11 having a diameter of 22.9 cm from tip to tip of the extending arms and 0.94 cm thick. The diffuser block 64 is made of mild steel (alloy 1010) and is 6.35 cm in diameter and 7.6 cm high. The magnet is a stacked pair of rare earth permanent magnets, each being Neo-37® magnet obtained from Dexter Magnetics and providing a magntic force of 3 tesla (30000 gauss). Each magnet It is 5.59 cm in diameter and 0.78 cm thick, and the stack of the two magnets is about 1.5 cm thick. Primer, midcoat and topcoat are applied to the cooking surface of the frying pan, in a similar manner as disclosed in Example 1, except that the primer layer is 7.5 micrometers thick, the midcoat layer is 18 micrometers thick and the topcoat is 5 micrometers thick, the thicknesses being controlled by the spray time used to apply the coatings. As in Example 1, the midcoat, which contains the magnetizable flakes is applied to the dry primer layer while being subjected to the magnetic force using the equipment arrangement just described. The three-coat system applied to the frying pan is baked as in Example 1 to obtain the pattern shown in Figure 12 wherein the dark appearing pattern in the release coating is set in a surrounding area of light-color, the dark-appearing pattern appearing to be recessed below the plane of the light color area, to give the cooking surface of the frying pan a three-dimensional appearance. The primer and topcoat compositions are similar to the corresponding compositions used in Example 1, and the midcoat composition was an aqueous dispersion having the following composition:

An mixture containing mixed aromatic hydrocarbons, cerium octoate, triethanolamine, oleic acid, Triton® X-100 surfactant in proportions to provide the composition in the following table is added to the blend of acrylic polymer dispersion and fluoropolymer dispersion. The stainless steel flakes, Cab-O-Sil® fumed silica, ethylene glycol, polyamic acid salt, sulfonate surfactant, Triton® X-100 surfactant, and furfural alcohol in proportions to provide the composition in the following table are milled together for addition to the blend of other components. The acrylic polymer dispersion corresponds to approximately to 39/57/4 (wt. ratio) methyl methacrylate/ethyl acrylate/methacrylic acid. The polymer comprises about 40% of the dispersion, 9% triethanolamine, 8% sodium lauryl sulfate, and the balance to total 100 wt% is water.

| **Component** | **Wet Composition (Wt. %)** | **Solids Content Coating in Finished Article (Wt. %)** |
|---|---|---|
| PTFE Dispersion | 57.15 | 80.3 |
| PFA Dispersion | 10.34 | 14.7 |
| Deionized Water | 4.96 | - |
| 316L SS Flake* | 1.8 | 4.3 |
| Solvent-Surfactant blend | 10.67 | - |
| Acrylic polymer dispersion | 12.7 | - |
| Polyamic acid salt in N-methyl pyrrolidone | 0.20 | 0.5 |
| Cab-O-Sil® fumed silica | 0.17 | 0.4 |
| sulfonate surfactant | 0.04 | - |
| Triton®X-100 surfactant | 0.68 | - |
| ethylene glycol | 0.04 | - |
| furfural alcohol | 0.02 | - |
| cerium octoate | 0.60 | - |
| diethyleneglycolmonobutylether | 2.51 | - |
| triethanolamine | 4.75 | - |
| 1,2,4-trimethylebenzene | 1.01 | - |
| cumene | 0.06 | - |
| xylene | 0.06 | - |
| aromatic hydrocarbon | 1.93 | - |
| Notes: The polyamic acid salt converts to polyamideimide upon baking. The wet composition contains 36% by weight of water, based on the total wet composition, the water coming primarily from the aqueous dispersion form of the PTFE and PFA. The overall water content of the total composition is 36% primarily supplied by the aqueous media from the polymer aqueous dispersions. | | |

| | | |
|---|---|---|
| *SS Fine water grade, -325 mesh with a D-50 = 25 micrometers (more than 50% of the particles have a longest dimension of at least 25 micrometers) produced by Novamet Specialty Products of Wyckoff, N.J. | | |

The polyamic acid salt in the composition provides the benefit of being compatible with both the SS flakes and the fluoropolymer components in the composition so that when the flakes reorient under the influence of magnetic force, the portions of the flakes which protrude above the flat surface of the midcoat will be enveloped by fluoropolymer, so that the reorientation does not produce minute fissures (visible under 20X magnification) in the midcoat during reorientation, i.e. tilting of the magnetically affected flakes from the horizontal towards the perpendicular may leave empty space being in the midcoat. Athough the midcoat is covered by a topcoat. minute fissues in the midcoat provide easy pathways for moisture to permeate through all the layers to reach the substrate (frying pan) and cause blistering of the coatings. Upon baking, the polyamic acid salt coverts to polyamideimide and bonds the flakes to the fluoropolymer. The midcoat obtained in this Example is free of minute fissures.

The surface of the baked coating on the frying pane is smooth to the touch, having a smoothness of about 0.8 micrometers in the light-colored area and about 1.3 micrometers in the pattern (dark color) area.

The importance of having the block 64 present to diffuse the magnetic force is indicated by reproducing this Example, but eliminating the block, whereby the magnet 66 is positioned in direct contact with the underside of plate 60. The resultant image is less sharp, and the surface of the baked coating (primer/midcoat/topcoat) is rougher, namely 1.75 to 2.5 micrometers in the pattern area), which compromises the release property of the coating.

## Claims

1. Process for forming a patterned release coating on a nonmagnetizable substrate, comprising
(a) applying a mixture of magnetizable flakes in a liquid dispersion of fluoropolymer onto said substrate to form a coating thereon,
(b) creating a diffuse magnetic field at a location spaced from said substrate,
(c) communicating magnetic force from said diffuse magnetic field through a magnetizable die pattern to said coating while still liquid to form a pattern of said flakes in said coating corresponding to the pattern of said die, and
(d) baking said coating to affix said pattern of flakes therein

2. The process of claim 1 wherein said magnetic force is communicated from sheet edges and/or pins forming the pattern of said die.

3. The process of claim 2 wherein said die having said sheet edges resembles a cookie cutter and the pattern of said flakes in said coating is a line pattern.

4. The process of claim 3 wherein said die comprises a plurality of pins wherein said pattern comprises a plurality of point corresponding to said pins.

5. The process of claim 1 wherein steps (a) and (c) are carried out simultaneously.
